

March 2, 1948.

J. SCHULEIN

2,436,940

METHOD OF REGENERATING ANODIZING BATHS

Filed Aug. 2, 1946

2 Sheets-Sheet 1



FIG. I.

INVENTOR.  
JOSEPH SCHULEIN  
BY  
Campbell, Brumit, Lang & Free  
his ATTORNEYS.

March 2, 1948.

J. SCHULEIN

2,436,940

METHOD OF REGENERATING ANODIZING BATHS

Filed Aug. 2, 1946

2 Sheets-Sheet 2



FIG. 2.

INVENTOR.  
JOSEPH SCHULEIN  
BY Campbell, Pennington & Free

his ATTORNEYS.

## UNITED STATES PATENT OFFICE

2,436,940

## METHOD OF REGENERATING ANODIZING BATHS

Joseph Schulein, Corvallis, Oreg.

Application August 2, 1946, Serial No. 688,038

15 Claims. (Cl. 204—130)

1

This invention relates to the treatment of chromic acid solutions to remove impurities therefrom and relates more particularly to the regeneration of spent chromic acid anodizing solutions.

This is a continuation-in-part of my abandoned applications Serial No. 494,772, filed July 15, 1943, and Serial No. 495,165, filed July 17, 1943.

Chromic acid anodizing solutions are commonly used in the treatment of aluminum and aluminum alloys to render the surfaces of the metal corrosion resistant. Large quantities of aluminum and aluminum alloys are treated by anodizing methods inasmuch as anodizing is a required treatment for the metal used in army and navy matériel.

The anodizing process includes the immersion of the metal in the anodizing solution and the use of the metal as an anode in an electrolytic process. The bath and the electric current convert the surface of the aluminum-containing metal into a mixture of aluminum oxide and aluminum hydroxide which protects the underlying metal because of the relative imperviousness and inertness of the oxide-hydroxide film.

The preferred type of anodizing solution, from the standpoint of optimum film-forming characteristics should contain about 10% chromic acid. A newly prepared chromic acid bath of that concentration will have a pH value of approximately 0.1. The exact pH value is dependent upon the concentration of chromic acid.

During the anodizing treatment, aluminum is dissolved from the surface of the material being treated and enters the bath, where it combines with some of the chromic acid to form aluminum dichromate. This compound is only slightly dissociated and, therefore, has the effect of decreasing the available chromic acid in the bath. The chromic acid that is combined in an undissociated state with the aluminum is commonly referred to as "fixed acid," while the chromic acid that is not combined in such an undissociated state is commonly referred to as "free acid."

Aluminum dichromate contains about 92% chromic acid and about 8% aluminum. Therefore, a small amount of aluminum dissolved in the bath causes a considerable decrease in the available free acid for the reason that it combines with about eleven times its own weight of chromic acid. Thus, for every pound of aluminum dissolved in the bath, 11 pounds of chromic acid are converted from the "free" state to the "fixed" state and become unavailable for continued formation of the anodic film.

2

It is the concentration of "free acid" that determines the acidity of the bath. Inasmuch as there is a definite relationship between the acidity of the bath and the characteristics and amount of anodic film produced, it is essential that the acidity of the bath be controlled within definite limits.

It has been found that the anodizing bath functions best if the acidity is kept within the range of pH 0.6 to pH 1.3. These pH conditions are commonly maintained by the periodic addition of chromic acid anhydride in an amount necessary to compensate for the chromic acid being "fixed" or combined in an undissociated state with the aluminum dissolved in the bath. The constant addition of chromic acid to the bath contributes to an ever-increasing concentration of total chromic acid in the bath. Under these conditions, the bath rapidly approaches a condition of extremely high density, and operating difficulties arise because of changes in electrical conductivity, viscosity, etc. Also, losses are encountered for the reason that as the work is removed from the bath, the liquid film adhering to the metal is of higher chromic acid concentration.

In order to compensate for these variations in the condition of the bath, it has been common practice to start a new bath at a low chromic acid concentration, such as 3 to 5%, and then add chromic acid to the bath as necessary, thereby prolonging the time until the chromic acid concentration becomes so high that the bath is no longer useful. Baths containing low concentrations of free chromic acid and baths containing a high "fixed" chromic acid concentration do not produce the best quality film. Therefore, quality of the anodic film has been sacrificed and non-uniformity of the film has resulted from the prior practice.

When the bath attains a concentration of "fixed acid" such that the use of the bath is no longer practical, the bath is discarded. Many thousands of gallons of spent chromic acid solutions have been discarded annually because of the above-described conditions.

An object of the present invention is to provide a method of treating chromic acid solutions containing "fixed acid" to convert the "fixed acid" into "free acid."

Another object of the invention is to provide a method of treating spent chromic acid anodizing solutions in order to recover the chromic acid therein and to permit the bath to be operated indefinitely.

Another object of the invention is to provide a method of regenerating chromic acid anodizing

baths to allow the operation of the bath within a narrow range of pH values and with only a small variation in the amount of "fixed" and "free" chromic acid in the bath, to cause the formation of more uniform anodic films.

Other objects of the invention will become apparent from the following description of typical methods of treating chromic acid solutions in accordance with the present invention.

In accordance with the present invention, chromic acid baths or solutions containing dissolved aluminum are treated to cause a conversion of the soluble aluminum dichromate therein into an insoluble aluminum compound and free chromic acid.

More particularly, the process includes the partial neutralization of chromic acid anodizing baths in order to convert the soluble aluminum dichromate into a form of aluminum dichromate which undergoes hydrolysis to form insoluble aluminum hydroxide and chromic acid. Thereafter, the solution may be filtered to eliminate the insoluble aluminum hydroxide and further treated to restore the bath to a desired pH value.

I have found that the conversion of the soluble aluminum dichromate into insoluble aluminum hydroxide and chromic acid takes place above a pH value of about 3. Preferably, the pH value should not be much below pH 3.5 if substantially complete separation of the aluminum ions is to be obtained. At a pH value of about 10, or above, some of the aluminum hydroxide will dissolve and moreover the chromic acid will be converted into a chromate. An excessive amount of alkali is required to neutralize the solution to higher pH values and no advantage is obtained thereby. Therefore, for practical purposes, neutralization of the anodizing bath to a pH value range of 3.5 to 5.0 is most advantageous.

The precipitate obtained in the pH value range of 3.5 to 5.0 may be regarded as aluminum hydroxide containing absorbed chromic acid. This precipitate may be filtered from the balance of the solution and washed with water at a maintained pH value higher than 3.5 so as to separate most of the absorbed chromic acid from the aluminum hydroxide as well as promote hydrolysis of any aluminum dichromate that may not have been hydrolyzed.

The filtrate is then treated to restore it to a desired pH value and may be treated further to eliminate unwanted ions introduced by the preceding treatments, whereby a purified bath is obtained with relatively little loss of chromic acid.

For a better understanding of the reactions involved, reference may be had to the accompanying drawing in which Figure 1 is a flow sheet of a typical process for regenerating chromic acid anodizing baths; and Figure 2 is a flow sheet of a modified process for regenerating such chromic acid anodizing baths.

In accordance with the present invention, and as illustrated in Figure 1, I withdraw a portion of the chromic acid solution from the anodizing bath 10 and deliver it to a tank 11 where it may be partially neutralized by the addition of calcium hydroxide, calcium carbonate or calcium oxide, or metallic calcium, thereby forming calcium dichromate in solution, plus an aluminum-containing precipitate. The amount of the calcium containing neutralizing agent should be sufficient to increase the pH value of the solution to about 3 or above, and preferably within a pH value range of 3.5 to 5, thereby converting the chromic acid to calcium dichromate and avoiding the forma-

tion of calcium chromate. In other words, the chromic acid should be about one-half neutralized by the addition of the lime.

After adjustment of the pH value and the formation of the aluminum-containing precipitate, the solution is passed to a filter 12 where the aluminum hydroxide precipitate is separated and washed. The filtrate is delivered to another tank 13 for further treatment.

A sufficient amount of sulphuric acid is added to the filtrate in the tank 13 to convert the calcium dichromate into chromic acid and insoluble calcium sulphate. The solution may be adjusted to a value between about pH 0.6 and pH 1.3, as desired, by the addition of sulfuric acid. This mixture is passed to the filter 14, thereby removing most of the calcium sulphate and recovering a filtrate of chromic acid that may be returned to the anodizing bath 10.

This process may be used for the treatment of an entire bath of the chromic acid solution or it may be used to regenerate portions of the bath so that the bath can be operated continuously within a narrow range of predetermined pH values. For example, after several days' operation, a portion of the bath containing an amount of aluminum equivalent to the amount of aluminum being dissolved in the entire bath each day may be removed and regenerated as described above. Thus, periodic treatment of small portions of the bath by the above-described method maintains the bath in constant operating condition.

The calcium sulphate precipitate, previously mentioned, is slightly soluble in the chromic acid solution, and, therefore, the solution which is returned to the anodizing bath contains a small amount of calcium sulphate.

If it is desired to reduce the amount of sulphate present in the anodizing bath, this may successfully be accomplished by treating the bath further before returning it to the bath. Thus, the filtrate from the filter 14 may be delivered to the receptacle 15 where barium carbonate is added to the solution in a quantity sufficient to react with the calcium sulphate to form barium sulphate which is less soluble than calcium sulphate. The calcium ions combine with the chromic acid to form calcium dichromate. The calcium dichromate has no effect on the anodizing bath other than using up a small amount of chromic acid in the "fixed" state.

The solution may be passed to the filter 16 to separate out the barium sulphate precipitate and the filtrate may then be returned to the anodizing bath.

The bath may be purified further by delivering the filtrate from the filter 16 to a receptacle 17, where hydrofluoric acid is added in an amount sufficient to precipitate the calcium in the form of calcium fluoride. The precipitated calcium fluoride is removed by the filter 18 and the filtrate containing a small amount of dissolved calcium fluoride is returned to the anodizing bath.

Upon adding the latter mixture to the anodizing bath, the calcium fluoride immediately reacts with the aluminum dichromate present in the bath to form calcium dichromate and aluminum fluoride, and undissociated compound which has no effect upon the operation of the anodizing bath.

While the process has been disclosed in the drawing in Figure 1 as a single flow sheet, it will be understood that the process may be practiced in part, or as a whole, as described.

By way of typical example of the process a sample was obtained from the anodizing bath used in the treatment of aluminum parts. The total chromic acid present was equivalent to 112 grams per liter of  $\text{CrO}_3$  of which 98 grams per liter was "fixed"  $\text{CrO}_3$  (combined with aluminum), and the remainder, 14 grams or 12½%, was free chromic acid. This sample was neutralized to a pH value of 4.27 with calcium hydroxide to cause precipitation of the aluminum as aluminum hydroxide. After filtration to separate the aluminum hydroxide precipitate, the filtrate was adjusted to a pH value of about 0.8 with sulphuric acid and filtered to remove calcium sulphate. Analysis of the filtrate showed that 99.3% of the "fixed" and "free" chromic acid was recovered as free chromic acid. Further treatment to remove sulphate and calcium ions by the addition of barium carbonate and hydrofluoric acid in the manner described above and in amounts chemically equivalent to the amount of calcium ions present, did not cause substantial loss of the free chromic acid.

While the process has been described with reference to the use of calcium hydroxide or lime as the neutralizing agent for the solution, it will be understood that neutralization and precipitation can be practiced with metallic calcium or calcium carbonate. The operations would be the same if these other materials were used in the proper equivalents or chemically stoichiometric proportions. Moreover, one or more of the steps of the process can be combined, if desired. For example, barium fluoride may be used instead of barium carbonate to reduce the amount of sulphate present, and to combine the precipitation of barium sulphate and calcium fluoride in one step.

The invention can be practiced in other ways also, thus, as described hereinafter a spent or contaminated anodizing bath can be treated to remove aluminum ions and thereafter treated electrolytically to remove unwanted metallic ions.

In accordance with the present invention and as illustrated in Figure 2, I withdraw a portion or all of the chromic acid solution containing aluminum dichromate from the anodizing bath 20 and deliver it to a tank 21 where it is partially neutralized by the addition of an alkaline agent whose metallic ion forms compounds that are soluble in the solution, such as, for example, sodium or potassium hydroxide, lime, calcium hydroxide or calcium carbonate. Sodium hydroxide is used, preferably, and the process will be described with reference to the use of sodium hydroxide as the alkaline agent. The addition of sodium hydroxide to the chromic acid solution results in the formation of sodium dichromate in solution, plus an aluminum-containing precipitate. The amount of sodium hydroxide or other alkaline agent should be sufficient to increase the pH value of the solution to about 3 or above and preferably within a pH value range of 3.5 to 5, thereby converting the chromic acid to sodium dichromate and avoiding the formation of sodium chromate. In other words, the chromic acid should be about one-half neutralized by the addition of the alkaline agent.

After adjustment of the pH value and the formation of an aluminum-containing precipitate, the solution is passed to a filter 22, where the aluminum hydroxide precipitate is separated out and washed with alkaline water to remove any sodium dichromate remaining in the precipitate.

The filtrate is delivered to storage tank 23 and thence to a diaphragm type of electrolytic cell 24 having an anode 25 on one side of the diaphragm 26 and a cathode 27 on the other side of the diaphragm.

When direct current is passed through the cell, the dichromate ions will be segregated as chromic or dichromic acid in the anolyte, and the sodium ions will be segregated in the catholyte, forming sodium hydroxide therein. The current and voltage used during electrolysis can be varied considerably, but preferably a current density and a voltage are used that will not cause excessive discharge of other ions, particularly hydrogen and oxygen, in amounts sufficient to effectively reduce the overall efficiency below a predetermined economic minimum taking into account the discharge potentials of these ions on various electrodes that may be used and the economic balancing of cell size and capacity at any given current density against initial and operating costs.

The chromic acid in the anolyte is returned to the anodizing bath. The sodium hydroxide solution is separated and is returned to a storage tank 28 for use in the neutralization of the next batch of anodizing solution.

A perfect separation of the sodium ions from the chromic acid solution or a complete separation of the chromic acid from the sodium hydroxide is not necessary as these solutions merely go around and around the circuit. The separation should be sufficiently complete, however, to maintain the anodizing bath within a pH value range of about 0.1 to 1.3.

As a specific example of the above process, a portion of an anodizing bath solution was neutralized to a pH value of 4.2 with sodium hydroxide and filtered. The filtrate contained 101.3 grams/liter  $\text{CrO}_3$  in the form of sodium dichromate. The filtrate was fed to an electrolytic cell. The electrolysis was conducted with a current of 0.5 ampere and a voltage of 15 to 18 was used to hold the current constant. After electrolysis, the anolyte liquor contained 95 grams/liter of free  $\text{CrO}_3$  and had a pH value of 0.13.

The recovery rate was 8.7 pounds of  $\text{CrO}_3$  per thousand ampere hours, which at a 3-volt cell drop is equivalent to 2.89 pounds of  $\text{CrO}_3$  per kilowatt hour.

From the preceding description, it will be clear that I have provided simple, yet effective methods of regenerating anodizing baths, whereby substantial economies are obtained in the anodizing operation and in the prevention of waste of a vital material. It will be understood that the processes can be varied considerably without departing from the invention, for example, all or a part of the bath may be treated periodically, the current densities used during electrolysis in accordance with the method illustrated in Figure 2 of the drawings can be varied and the pH value of the regenerated bath can be controlled as the purpose demands. Therefore, the above-described methods should be construed as illustrative and not as limiting the scope of the following claims.

I claim:

1. A method of regenerating a chromic acid anodizing solution having a pH value less than 3 and containing undissociated aluminum dichromate, which comprises adding an alkaline agent of the class consisting of sodium hydroxide, potassium hydroxide, lime, calcium hydroxide and calcium carbonate to said solution to increase its

pH value to not less than 3 and form an aluminum hydroxide precipitate, separating said precipitate from said solution, and thereafter removing the metal ions of said alkaline agent to adjust the pH value of said solution to less than 1.3.

2. A method of regenerating a chromic acid anodizing solution having a pH value less than 3 and containing undisassociated aluminum dichromate, which comprises adding lime to said solution to increase its pH value to between about 3.5 and 5.0 and form an aluminum hydroxide precipitate, separating said precipitate from said solution, and thereafter removing the metal ions of said alkaline agent to adjust the pH value of said solution to a pH value of less than 1.3.

3. A method of regulating the pH value of a chromic acid anodizing bath containing aluminum dichromate which comprises withdrawing a portion of said bath, adjusting the pH value of the portion to not less than 3 with sodium hydroxide to form an aluminum hydroxide precipitate, removing said precipitate from said portion, thereafter electrolyzing said portion in a diaphragm cell to form an anolyte having a pH value between about 0.1 and 1.3 and mixing said anolyte with the remainder of said bath.

4. A method of regulating the pH value of a chromic acid anodizing bath containing aluminum dichromate which comprises withdrawing a portion of said bath, adjusting the pH value of said portion to between about 3.5 and 5.0 with an alkaline agent of the class consisting of sodium hydroxide, potassium hydroxide, lime, calcium hydroxide and calcium carbonate, removing from said portion any aluminum-containing precipitate formed therein, thereafter electrolyzing said portion in a diaphragm cell to form an anolyte having a pH value between about 0.1 and 1.3 and mixing said anolyte with the remainder of said bath.

5. A method of regulating the pH value of a chromic acid anodizing bath containing aluminum dichromate which comprises withdrawing a portion of said bath, adjusting the pH value of said portion to between about 3.5 and 5.0 with sodium hydroxide, removing from said portion any aluminum-containing precipitate formed therein, thereafter electrolyzing said portion in a diaphragm cell to form an anolyte having a pH value between about 0.1 and 1.3 and mixing said anolyte with the remainder of said bath.

6. A method of maintaining within an optimum operating range the pH value of a chromic acid bath for anodizing aluminum-base metals and which contains undisassociated, soluble aluminum dichromate, which comprises withdrawing a portion of said bath when said bath attains a pH value of about 1.3, adjusting the pH value of said portion to not less than 3 with an alkaline agent of the class consisting of sodium hydroxide, potassium hydroxide, calcium hydroxide, lime and calcium carbonate, to form a precipitate of aluminum hydroxide, separating said precipitate from said portion, thereafter electrolyzing said portion in a diaphragm cell to form an anolyte having a pH value of less than 1.3, and mixing said anolyte with the remainder of said bath.

7. A method of maintaining the pH value of a chromic acid bath for anodizing aluminum-base metals within an optimum operating range of pH values not exceeding about 1.3, said bath containing undisassociated aluminum dichromate, which comprises withdrawing a portion of said bath when said bath attains a pH value of about

1.3, adjusting the pH value of said portion with sodium hydroxide to not less than 3, to form a precipitate of aluminum hydroxide, separating said precipitate from said portion, thereafter electrolyzing said portion in a diaphragm cell to form an anolyte having a pH value of less than 1.3, and mixing said anolyte with the remainder of said bath.

8. A method of maintaining the pH value of a chromic acid bath for anodizing aluminum-base metals within an optimum operating range of about 0.6 to 1.3, said bath containing soluble aluminum dichromate, which comprises withdrawing at least a portion of said bath when said bath attains a pH value as high as the highest pH value set for the optimum operating range, adjusting the pH value of said portion to not less than 3 with an alkaline agent of the class consisting of sodium, potassium and calcium hydroxides, lime and calcium carbonate, to form a precipitate of aluminum hydroxide, separating said precipitate from said portion, thereafter electrolyzing said portion to form an anolyte having a pH value within said optimum operating range, and mixing said anolyte with the remainder of said bath.

9. A method of controlling the pH value of a chromic acid bath for anodizing aluminum-containing articles, comprising segregating a portion of said bath, adding lime to said portion to adjust the pH value of said portion to at least 3.0 and precipitate an aluminum compound in said portion, filtering said portion to remove the insoluble aluminum compound, adding sulfuric acid to the filtrate to adjust its pH value to between about 0.6 and 1.3, removing any precipitate formed thereby and adding the filtrate to the remainder of said bath.

10. A method of controlling the pH value of a chromic acid bath for anodizing aluminum-containing articles, comprising segregating a portion of said bath, adding lime to said portion to adjust the pH value of said portion to at least 3.0 and precipitate an aluminum compound in said portion, filtering said portion to remove the insoluble aluminum compound, adding sulfuric acid to the filtrate to adjust its pH value to between about 0.6 and 1.3 removing any precipitate formed thereby, adding a soluble barium compound to said filtrate, removing any precipitate formed thereby, and adding the filtrate to the remainder of said bath.

11. A method of controlling the pH value of a chromic acid bath for anodizing aluminum-containing articles, comprising segregating a portion of said bath, corresponding substantially to the amount of aluminum dissolved in said bath in a predetermined period, adding lime to said portion to adjust the pH value of said portion to at least 3.0 and precipitate an aluminum compound in said portion, filtering said portion to remove the insoluble aluminum compound, adding sulfuric acid to the filtrate to adjust its pH value to between about 0.6 and 1.3, removing any precipitate formed thereby, and adding the filtrate to the remainder of said bath.

12. A process for regenerating a chromic acid solution from an anodizing bath for aluminum and aluminum base alloys comprising adding lime to adjust the acidity of the solution to a pH value greater than 3.0 to form a precipitate, removing said precipitate, and adding sulphuric acid to said solution to reduce its pH value to not more than about 1.3.

13. A process for regenerating a chromic acid

solution from an anodizing bath for aluminum-containing articles comprising adding lime to said solution to adjust its acidity to a pH value greater than 3.0, filtering said solution, readjusting the acidity of the filtrate by the addition of sulphuric acid, filtering the adjusted solution, treating the filtrate from the adjusted solution with barium carbonate, removing any precipitate formed thereby, adding hydrofluoric acid to the resulting solution and removing the precipitate formed thereby.

14. A process for regenerating a chromic acid solution from an anodizing bath for aluminum-containing articles, comprising adding lime to said solution to adjust its acidity to a pH value greater than 3.0, removing any precipitate formed thereby, adding sulphuric acid to the solution to reduce its pH value to less than 1.3, removing any further precipitate formed thereby, and adding barium fluoride to said solution.

15. A process for regenerating a chromic acid solution from an anodizing bath for aluminum-containing articles, comprising adding lime to the solution to adjust its acidity to a pH value between about 3.5 and 5.0 to form a precipitate, removing said precipitate, adding sulphuric acid to the solution to separate calcium ions as calcium sulfate, removing said calcium sulfate, adding barium

fluoride and removing any precipitate formed thereby.

JOSEPH SCHULEIN.

#### REFERENCES CITED

The following references are of record in the file of this patent:

#### UNITED STATES PATENTS

|    | Number    | Name                 | Date           |
|----|-----------|----------------------|----------------|
| 10 | 1,857,548 | Humphries -----      | May 10, 1932   |
|    | 1,954,664 | Cain -----           | Apr. 10, 1934  |
|    | 2,055,961 | Boss -----           | Sept. 29, 1936 |
|    | 2,081,787 | Boss -----           | May 25, 1937   |
| 15 | 2,099,658 | Pearson et al. ----- | Nov. 16, 1937  |
|    | 2,159,074 | Briggs -----         | May 23, 1939   |
|    | 2,316,750 | Ambrose -----        | Apr. 20, 1943  |

#### FOREIGN PATENTS

|    | Number  | Country             | Date          |
|----|---------|---------------------|---------------|
| 20 | 144,710 | Great Britain ----- | Jan. 13, 1921 |
|    | 644,077 | France -----        | May 26, 1928  |

#### OTHER REFERENCES

- 25 Monthly Review of the American Electroplaters Society, Oct. 1942, pages 831 through 837.  
Hackh's Chemical Dictionary, 2d edition (1937), page 543 ("Lime").